

J. TERWELP.

PROCESS FOR THE DIRECT PRODUCTION OF PURE OXID OF TIN  
APPLICATION FILED SEPT. 3, 1914.

1,237,840.

Patented Aug. 21, 1917.

FIG. 1.



FIG. 2.



FIG. 3.



Witnesses:

B. Dammers  
E. Leekens

Inventor:

Johann Terwelp  
Signature

Attest:

# UNITED STATES PATENT OFFICE.

JOHANN TERWELP, OF NEUSS, GERMANY.

## PROCESS FOR THE DIRECT PRODUCTION OF PURE OXID OF TIN.

1,237,840.

Specification of Letters Patent. Patented Aug. 21, 1917.

Application filed September 3, 1914. Serial No. 860,063.

*To all whom it may concern:*

Be it known that I, JOHANN TERWELP, chemist, a subject of the German Emperor, and residing at Neuss, Rhine, Germany, have invented certain new and useful Processes for the Direct Production of Pure Oxid of Tin, of which the following is a specification.

The object of the present invention relates to the production of pure oxid of tin, immediately fit for the production of enamel from tin-bearing materials of any kind. Preferably the oxid of tin, precipitated from the sodium stannate solutions in connection with the freeing of white metal from tin (which oxid of tin has a mean percentage of from about 90 to 95%  $\text{SnO}_2$ ) or the tin paste, obtained in the dyeing of silks (which paste has a percentage of from about 85% to 95%  $\text{SnO}_2$ ) can be used as starting materials.

The process consists in heating first the tin bearing material to approximately the reduction-temperature of the oxid of tin. The temperature may, however, also be higher but not so high, that the tin-bearing material comes to a melt. While retaining the temperature of heating and in presence of an oxidizing atmosphere, a reducing agent is gradually supplied to the material, heated in this way. To this effect gaseous and finely distributed liquid reducing agents, such as *e. g.* lighting gas or oil, or else solid reducing agents, such as finely powdered carbon or its equivalents are used. The latter reducing agents are conveniently fed by means of an atomizing nozzle or with the assistance of such devices, as are made use of for the combustion of coal dust in connection with coal dust-furnaces. The reducing agent is gradually fed on the heated material only until all the tin has been converted into oxid of tin. In this manner an exceedingly pure and light oxid of tin is obtained in finely distributed condition.

For carrying out the present process nothing is required but a device for heating the material to be treated, and a device for feeding the reducing agent and the oxidizing air or the like and finally a device for gathering the oxid of tin produced.

A practical form of embodiment of a device by means whereof the present process can be carried into effect is exemplified on the accompanying drawing, wherein Figure 1 shows a flame-furnace closed on top, in

longitudinal section; Fig. 2 is a section on the line A—B of Fig. 1; Fig. 3 represents a section through the line C—D of Fig. 1.

The flame-furnace *a* has a hearth *b*, on which the tin-bearing material to be dealt with is charged through the opening *c*. As soon as the material is placed on the hearth and the furnace is started, such opening is hermetically closed by a plate *d*. The tin-bearing material in the furnace is heated to about 1000° to 1100° C. by means of large Bunsen burners *e*. Now, while retaining the temperature, the reducing agent, in presence of an oxidizing atmosphere, is allowed gradually to act on the surface of the glowing material, heated in this manner. When applying lighting gas as reducing-agent and air as an oxidizing-agent, the Bunsen-burners *e* are used to supply a mixture of lighting gas and air, rarefied by air, which mixture can be supplied to the burners by means of any suitable device. During this phase of the process it will be well to stop some of the Bunsen burners *e* with a view of avoiding an increase in temperature during the production of oxid of tin. When liquid or solid reducing agents are used, they are fed in a similar manner, by blowing the reducing agent in finely distributed form together with an air current on the material to be treated.

The oxid of tin, obtained in form of vapors in presence of an oxidizing atmosphere during the action of the reducing agent, escapes from the opening *f* into a conduit *g*, which conveniently slightly ascends and is connected with the furnace. In front of the opening *h* of this conduit a chimney-like structure *i*, open at its base and allowing inspection of the conduit, is placed. From the upper end thereof a pipe *k* leads toward the settling chambers and collectors, where-in the ready product is gathered.

### Example.

100 kgs. of tin paste or residue, from the dyeing of silk and composed of about 93% of oxid of tin, sand and further mechanical impurities are finely pulverized and heated up to approximately 1000 to 1100° C. in the flame-furnace, without any admixture. Now, while retaining the temperature, lighting gas is conveyed from a pipe provided with a regulating device and simultaneously therewith air by means of an air-compressor, testing to a pressure of water-column of

from 1000 to 1200 mm., is forced into the furnace chamber above the surface of the heated material. Under the temperature maintained in the furnace and in presence 5 of the oxidizing air, one portion of the oxid after the other is reduced on the surface of the tin-bearing material, and oxidized again *in statu nascendi*, the product formed escaping as oxid. All that is necessary is to 10 regulate during the process the addition of the reducing agent so that all the tin that is formed is fully oxidized. In this manner a very voluminous, white product having a percentage of approximately 99% of  $\text{SnO}_2$ , 15 is obtained, this being particularly fit for enameling purposes.

What I claim is:—

- 20 1. The process of directly producing pure oxid of tin from tin bearing materials, which comprises heating the material to at least the reduction temperature of tin oxid without producing a melt, in the presence of a reducing agent, in an oxidizing atmosphere, whereby the tin vapor is immediately oxidized and leaves the charge as oxid fumes.
- 25 2. The process of directly producing pure tin oxid from tin bearing materials, which comprises heating the material without admixture of reducing agent to or above the

reduction temperature of tin oxid, and directing onto the surface of the charge a reducing agent in an oxidizing atmosphere. 30

3. The process of directly producing pure oxid of tin from tin bearing materials, which comprises heating the material to at least 35 the reduction temperature of the material without a reducing agent and supplying a gaseous reducing agent to the material in the presence of air sufficient to oxidize the tin vapor resulting from the reducing action. 40

4. The process of directly producing pure oxid of tin from tin bearing materials, which comprises heating the materials sufficiently to reduce them, and supplying to the material a mixture of reducing material and air 45 in an oxidizing atmosphere.

5. The process of directly producing pure oxid of tin from tin bearing materials, which comprises heating the materials sufficiently to reduce them, and supplying to the surface 50 of the material a mixture of reducing material and air in an oxidizing atmosphere.

In testimony whereof, I affix my signature in the presence of two witnesses.

JOHANN TERWELP. [L.S.]

Witnesses:

HELEN NUFER,  
ALBERT NUFER.